

1

3,006,937

ESTER OILS AND PROCESS FOR THEIR  
PREPARATION

Karl Büchner, Duisburg-Hamborn, and Heinrich Schwarz,  
Oberhausen-Sterkrade, Germany, assignors to Ruhr-  
chemie Aktiengesellschaft, Oberhausen-Holten, Ger-  
many, a corporation of Germany  
No Drawing. Filed Dec. 15, 1953, Ser. No. 398,416  
Claims priority, application Germany Dec. 18, 1952  
14 Claims. (Cl. 260—410)

This invention relates to new and useful improvements in ester oils.

One object of the invention is valuable ester oils having a low pour point. This, and still further objects will become apparent from the following description:

In accordance with the invention it has been found that esters having a hydroaromatic component and an aliphatic component constitute valuable oils which have a low pour point. These oils have proven particularly suitable as clock-work oil or lubrication oil for ice machines, and other machines and apparatus which operate at low temperature. The oils have also proven particularly valuable when used alone or in mixture, as circulating oils for turbines or for breaking-in oils for internal combustion engines. Depending upon the chain length of the aliphatic ester portion, the flash point of these oils may be adjusted to the particular level desired, while the pour point, especially in the case of high-molecular weight aliphatic portions, may be kept low by chain branching.

The ester oils in accordance with the invention may be esters of hydroaromatic alcohols and aliphatic carboxylic acids or of hydroaromatic carboxylic acids and aliphatic alcohols. It has been found that if the carbonyl group in the ester is located on the aliphatic side, i.e., the esters are esters of aliphatic carboxylic acids and hydroaromatic alcohols, particularly good viscosity indexes will be obtained.

The hydroaromatic ester components are preferably obtained by the catalytic addition of water gas to terpene hydrocarbons ( $C_{10}H_{16}$ ) as, for example, are available in turpentine oil.

The catalytic addition of water gas, i.e., carbon monoxide and hydrogen to the terpene hydrocarbons is the conventional aldehyde synthesis and is effected, for example, with cobalt catalysts. The catalysts, gas pressures and temperatures used therein are those as known to any expert familiar with the Oxo synthesis or hydroformylation (see, for example, U.S. Patents 2,327,066, 2,497,303; U.K. Patent 614,010; FIAT Report No. 1000; "Petroleum Processing," February 1953, pp. 241-248). The starting terpene hydrocarbon may constitute the total terpenes or individual fractions of a narrow boiling range. When individual fractions are used, the same may be processed or pretreated with catalysts in the conventional manner for the purpose of rearrangement or cyclization.

The addition products from the catalytic water gas addition may be converted into carboxylic acids or alcohols.

The addition products may be converted into carboxylic acids by oxidation, as, for example, with air or oxygen, or may be converted into carboxylic salts by the addition of mild alkali. The carboxylic acids may be recovered from these salts in the known manner.

The addition products may be converted into alcohols by catalytically hydrogenating the same, or, if desired, by using a hydrating hydrogenation in the known manner for obtaining a higher yield. The alcohols may be used as such or may be converted into corresponding carboxylic acids by treatment with alkali at the melting temperature in the conventional manner.

The starting materials of the process according to the

2

invention are terpene hydrocarbons of the general formula  $C_{10}H_{16}$  known under the collective term of terpene. This includes both, the hydrocarbon camphene and the isomeric hydrocarbon dipentene. The difference between the two hydrocarbons is that the former (camphene) is bicyclic and monoolefinic and the latter (dipentene) is monocyclic and diolefinic.

Camphene has the following structural formula:



10

15

30

35

45

50

55

60

70

By the catalytic addition of water gas (Oxo synthesis) followed by hydrogenation, there is formed therefrom the terpanol (camphanol) having the following structural formula:



It is possible by oxidation to recover from terpanol of the above structure the terpane-carboxylic acid (camphane carboxylic acid) having the following structural formula:



The dipentene which is isomeric with the camphene has the following structural formula:



Herefrom, by the catalytic addition of water gas followed by hydrogenation, an isomeric terpanol (menthane-methylol) is recovered having the following structural formula:

Herefrom, by oxidation, the corresponding terpane car-

boxylic acid may be recovered which has the following structural formula:



If the hydroaromatic portion is present as an alcohol, fatty acids must, of course, be used for the esterification. Alcohols or carboxylic acids of the molecular size  $C_2$  to  $C_{20}$  and preferably  $C_4$  to  $C_{18}$  are used for the esterification. The esterification is effected by methods known to any expert which is familiar with the esterification of organic compounds. The esterification conditions used may be seen in detail from the following examples. The use of short-chain acids results in esters of low viscosity having flash points of about  $117$ – $150$ ° C.; pour points below  $-60$ ° C., and high viscosity indexes. The characteristics of such esters are as follows:

|                                      | Density at 20° C. | $n_D^{20}$ | Ester number | Pour point °C. | Flash point °C. | Viscosity at 30° C. | Viscosity index |
|--------------------------------------|-------------------|------------|--------------|----------------|-----------------|---------------------|-----------------|
| Terpane methylol/ester acetic acid   | 0.965             | 1.4640     | 264          | -66            | 117             | 1.44                | +155            |
| Terpane methylolpropionic acid ester | 0.958             | 1.4634     | 248          | -68            | 124             | 1.43                | +164            |
| Terpane methylolbutyric acid ester   | 0.947             | 1.4631     | 234          | -70            | 129             | 1.51                | +152            |
| Terpane methylolvaleric acid ester   | 0.939             | 1.4612     | 220          | -68            | 144             | 1.64                | +148            |
| Terpane methylolcaproic acid ester   | 0.93              | 1.4631     | 202          | -71            | 153             | 1.77                | +157            |

If the esterification is effected with long-chain fatty acids, ester oils of increased viscosity and having flash points which range above  $200$ ° C., are obtained. The viscosity index of these oils ranges above 125. The pour points of these oils, however, are relatively high, so that the same are not high-grade lubricating oils. For example, the stearic ester of terpane methylol  $C_{11}H_{20}O$  has the following characteristics:

|                              |           |
|------------------------------|-----------|
| Density at 20° C.            | 0.907     |
| Refractive index $n_D^{20}$  | 1.4666    |
| Ester number                 | 124 (129) |
| Flash point °C.              | 216       |
| Viscosity at 30° C. ° Engler | 4.67      |
| Viscosity index              | 138       |
| Pour point °C.               | +12       |

If, instead of unbranched fatty acids, branched chain fatty acids are used, as, for example, a branched  $C_{15}$  fatty acid, then ester oils are obtained which meet all the requirements of the highest grade lubricants. An ester lubricating oil of this kind has the following characteristics, for example:

|                              |        |
|------------------------------|--------|
| Density at 20° C.            | 0.910  |
| Refractive index, $n_D^{20}$ | 1.4666 |
| Viscosity:                   |        |
| At 30° C. Engler degrees     | 3.77   |
| At 50° C. do                 | 2.17   |
| At 80° C. do                 | 1.48   |
| Flash point °C.              | 218    |
| Pour point °C.               | -58    |
| Viscosity index              | 120    |
| Saponification number        | 136    |
| Molecular weight             | 390    |

If the hydroaromatic component of the ester is in the form of the acid, then, instead of the terpane methylol, the corresponding terpane carboxylic acid  $C_{11}H_{18}O_2$  may be used. This terpane carboxylic acid may be obtained as an oxidation product of the terpane methylol. The terpane carboxylic acid may also be obtained from the terpane methylol formed by the catalytic addition of the

water gas to the terpene hydrocarbon by treatment with oxygen or air, if necessary or desired, in the presence of mild alkali, such as soda. When using the hydroaromatic component in the form of a carboxylic acid, the aliphatic component must, of course, be in the form of an alcohol. The same considerations should be given when choosing the alcohol as indicated above for the aliphatic carboxylic acid. Thus, branched aliphatic alcohols should be used in the case of long-chain compounds in order to keep the pour point low. Branched alcohols of this type are obtained, for example, by the catalytic addition of carbon monoxide and hydrogen to olefins, followed by a catalytic treatment with hydrogen if in the fractional distillation of the hydrocarbon-alcohol mixtures the first third or first four-tenths of the distillate are collected separately from the remainder. The intermediate fraction obtained between the hydrocarbon fraction and the alcohol may also be used for the production of the ester oils of low pour point in accordance with the invention. Esters thus produced, however, have the carbonyl group separated by an oxygen bridge on the hydroaromatic ester side. As indicated in Examples 5, 6, and 7 of the following examples, esters of this type exhibit a poorer viscosity index, and their flash points are lower by 10–20° C. than

those of the corresponding esters produced from terpane methylol and branched fatty acids.

The esters themselves may be distilled under reduced pressure without decomposition and are easily obtained in this manner in pure form.

The following examples are given by way of illustration and not limitation:

#### Example 1

336 grams (2 mols) terpane methylol  $C_{11}H_{20}O$ , which had been obtained from turpentine oil by the catalytic addition of water gas and by hydrogenation, were boiled with 130 grams acetic anhydride, 1 cc. concentrated hydrochloric acid and 150 cc. benzene for 2 hours under a reflux condenser with water separator. Thereafter, the raw product was washed three times with the same volume of water and the benzene was distilled off. A raw ester having the following characteristics was obtained:

|                              |                        |
|------------------------------|------------------------|
| Acid number                  | 0.                     |
| Ester number                 | 255 (calculated: 267). |
| Hydroxyl number              | 0.                     |
| Density at 20° C.            | 0.965.                 |
| Refractive index, $n_D^{20}$ | 1.4632.                |
| Molecular weight             | 204 (calculated: 210). |

Distillation resulted in a water-white ester having a boiling point of  $119$ – $132$ ° C. at 10 mm. Hg and having the following characteristics:

|                              |                        |
|------------------------------|------------------------|
| Acid number                  | 0.                     |
| Ester number                 | 264 (calculated: 267). |
| Hydroxyl number              | 0.                     |
| Density at 20° C.            | 0.965.                 |
| Refractive index, $n_D^{20}$ | 1.4640.                |
| Molecular weight             | 212 (calculated: 210). |
| Pour point                   | -66° C.                |
| Flash point                  | 117° C.                |
| Viscosity index              | 155.                   |

#### Example 2

75 The same mixture as used in Example 1 was used for

the esterification with the exception that 180 grams commercial propionic acid were used instead of 130 grams acetic anhydride. During the esterification, a quantity of propionic acid equivalent to the acid content of the separated water was added. After the distillation, a water-white ester boiling between 129 and 141° C. at 10 mm. Hg, and having the following characteristics, was obtained:

|                              |                        |
|------------------------------|------------------------|
| Acid number                  | 0.                     |
| Ester number                 | 248 (calculated: 250). |
| Hydroxyl number              | 0.                     |
| Density at 20° C.            | 0.958.                 |
| Refractive index, $n_D^{20}$ | 1.4634.                |
| Molecular weight             | 220 (calculated: 224). |
| Pour point                   | 68° C.                 |
| Flash point                  | 124° C.                |
| Viscosity index              | 164.                   |

#### Example 3

The same mixture as used in Example 1 was subjected to the esterification with the use of 210 grams commercial butyric acid instead of 130 grams acetic acid. The addition of butyric acid during the esterification was not necessary. A water-white ester boiling between 142° and 154° C. at 10 mm. Hg and having the following characteristics was obtained:

|                              |                        |
|------------------------------|------------------------|
| Acid number                  | 0.                     |
| Ester number                 | 234 (calculated: 235). |
| Hydroxyl number              | 0.                     |
| Density at 20° C.            | 0.947.                 |
| Refractive index, $n_D^{20}$ | 1.4631.                |
| Molecular weight             | 241 (calculated: 238). |
| Pour point                   | 70° C.                 |
| Flash point                  | 129° C.                |
| Viscosity index              | 152.                   |

#### Example 4

The valeric acid ester and caproic acid ester were produced in the manner described in the preceding examples with the use of commercial valeric acid and caproic acid, respectively. To remove the excess acid, the raw esters were washed, prior to the washing with water, with a 2% caustic soda solution until the acid number had dropped to 0. At 143° C. and 5 mm. Hg a valeric acid ester was obtained which had the following characteristics:

|                              |                        |
|------------------------------|------------------------|
| Acid number                  | 0.                     |
| Ester number                 | 220 (calculated: 222). |
| Hydroxyl number              | 0.                     |
| Density at 20° C.            | 0.939.                 |
| Refractive index, $n_D^{20}$ | 1.4612.                |
| Molecular weight             | 253 (calculated: 252). |
| Pour point                   | 68° C.                 |
| Flash point                  | 144° C.                |
| Viscosity index              | 148.                   |

The corresponding caproic acid ester which had a boiling point of 138° C.-140° C. at 0.8 mm. Hg had the following characteristics:

|                              |                        |
|------------------------------|------------------------|
| Acid number                  | 0.                     |
| Ester number                 | 202 (calculated: 210). |
| Hydroxyl number              | 0.                     |
| Density at 20° C.            | 0.934.                 |
| Refractive index, $n_D^{20}$ | 1.4631.                |
| Molecular weight             | 263 (calculated: 266). |
| Pour point                   | 71° C.                 |
| Flash point                  | 153° C.                |
| Viscosity index              | 157.                   |

#### Example 5

200 grams terpane methylol were boiled with 242 gms. of  $C_{15}$  fatty acid, which had been produced by treating a branched  $C_{15}$  alcohol having a pour point of -29° C.

with alkali at melting temperature, in the presence of 150 cc. toluene and 1 cc. concentrated hydrochloric acid under a reflux condenser with water separation in the manner described in Example 1. After two hours, the raw product was washed with water to remove the hydrochloric acid and distilled. After the removal of the toluene and of the excess terpane methylol, there was obtained as the main fraction at 208°-210° C. and 0.8 mm. Hg a viscous ester which had the following characteristics:

|                              |                        |
|------------------------------|------------------------|
| Acid number                  | 0.                     |
| Ester number                 | 136 (calculated: 143). |
| Hydroxyl number              | 0.                     |
| Density at 20° C.            | 0.910.                 |
| Refractive index, $n_D^{20}$ | 1.4666.                |
| Molecular weight             | 390 (calculated: 392). |
| Pour point                   | 58° C.                 |
| Flash point                  | 218° C.                |
| Viscosity at 50° C.          | 2.165 Engler degrees.  |
| Viscosity index              | 132.                   |

#### Example 6

228 grams of a branched  $C_{15}$  alcohol having the characteristics:

|                                                                                                                                                        |                        |
|--------------------------------------------------------------------------------------------------------------------------------------------------------|------------------------|
| Hydroxyl number                                                                                                                                        | 230                    |
| Pour point                                                                                                                                             | 30° C.                 |
| Density at 20° C.                                                                                                                                      | 0.840                  |
| 202 gms. of terpane carboxylic acid produced by treating terpane methylol with alkali at melting temperature and having the following characteristics: |                        |
| Acid number                                                                                                                                            | 298 (calculated: 308). |
| Density at 20° C.                                                                                                                                      | 1.015.                 |
| Refractive index, $n_D^{20}$                                                                                                                           | 1.4778.                |
| Pour point                                                                                                                                             | 22°C.                  |

200 cc. toluene and 3 gms. of toluene-sulfonic acid were boiled for 3 hours at a reflux condenser with water separation. Following this, the raw product was washed at first with a 2% caustic soda solution until the acid number had disappeared, and then with 50% ethyl alcohol to wash out dissolved soaps. Then it was distilled. At 208°-217° C. and 1 mm. Hg the pure ester was obtained which had the following characteristics:

|                              |                        |
|------------------------------|------------------------|
| Acid number                  | 0.                     |
| Ester number                 | 129 (calculated: 143). |
| Hydroxyl number              | 0.                     |
| Density at 20° C.            | 0.907.                 |
| Refractive index, $n_D^{20}$ | 1.4670.                |
| Molecular weight             | 398 (calculated: 392). |
| Pour point                   | 60° C.                 |
| Flash point                  | 195° C.                |
| Viscosity at 50° C.          | 2.24 Engler degrees.   |
| Viscosity index              | 96.                    |

The flash point of this ester was lowered by 23° C. and the viscosity index was lower by 36 units as compared with the corresponding ester prepared in accordance with Example 5.

#### Example 7

150 gms. of a synthetic branched  $C_{12}$  alcohol having the characteristics:

|                                                                                                               |                            |
|---------------------------------------------------------------------------------------------------------------|----------------------------|
| Molecular weight                                                                                              | 186.                       |
| Hydroxyl number                                                                                               | 300.                       |
| Pour point                                                                                                    | -53° C.                    |
| Boiling range                                                                                                 | 131°-134° C. at 10 mm. Hg. |
| were esterified with 180 gms. of terpane carboxylic acid in accordance with Example 6. The ester obtained had |                            |
| 70 the following characteristics:                                                                             |                            |
| Density at 20° C.                                                                                             | 0.918.                     |
| Refractive index, $n_D^{20}$                                                                                  | 1.4653.                    |
| Ester number                                                                                                  | 162 (calculated: 160).     |
| Hydroxyl number                                                                                               | 0.                         |

|                    |                        |
|--------------------|------------------------|
| Acid number        | 0.                     |
| Molecular weight   | 351 (calculated: 350). |
| Pour point         | -59° C.                |
| Flash point        | 185° C.                |
| Viscosity at 30° C | 2.96 Engler degrees.   |
| Viscosity at 50° C | 1.87 Engler degrees.   |
| Viscosity index    | 125 Engler degrees.    |

The same C<sub>12</sub> alcohol was subjected to the treatment with alkali at melting temperature and then to a treatment with acid, thereby producing the branched C<sub>12</sub> fatty acid which had the following characteristics:

|                              |                        |
|------------------------------|------------------------|
| Density at 20° C             | 0.891.                 |
| Refractive index, $n_D^{20}$ | 1.4387.                |
| Acid number                  | 278 (calculated: 279). |
| Pour point                   | -40° C.                |

222 gms. (1.11 mols) of this acid were esterified with 151 gms. (0.9 mol) terpane methylol with the addition of toluene as described in the preceding examples. After the separation of 16 cc. (0.89 mol) of water, the excess acid was removed by washing with 5% aqueous caustic soda solution and 50% ethanol and the raw ester was fractionated. The ester thus obtained in the pure form had the following characteristics:

|                              |                          |
|------------------------------|--------------------------|
| Density at 20° C             | 0.910.                   |
| Refractive index, $n_D^{20}$ | 1.4641.                  |
| Ester number                 | 162 (calculated: 160).   |
| Hydroxyl number              | 0.1.                     |
| Molecular weight             | 350.5 (calculated: 350). |
| Pour point                   | -64° C.                  |
| Flash point                  | 199° C.                  |
| Viscosity at 30° C           | 2.72 Engler degrees.     |
| Viscosity at 50° C           | 1.775 Engler degrees.    |
| Viscosity index              | 129.                     |

#### Example 8

370 grams (2.2 mols) terpane methylol C<sub>11</sub>H<sub>20</sub>O were boiled with 564 grams (2 mols) commercial oleic acid and 180 cc. commercial toluene, to which 3 grams p-toluene-sulfonic acid had been added, for 2 hours in a 2 liter round-bottomed flask with reflux condenser and water separation. During this time, 36 cc. of water which, by azeotropic distillation of the toluene, had been removed from the esterification mixture, accumulated in the water separating vessel. After the termination of the water separation, the toluene was removed from the esterification mixture by distillation under atmospheric pressure. Following this, the excess terpanol was removed by distillation under reduced pressure of about 10-1 mm. Hg at a temperature of 100°-130° C.

The residue from distillation was now mixed with 8.6 grams magnesia and distilled at 0.4 mm. Hg and bottom temperatures of 225-260° C. in a high-vacuum apparatus with short distilling paths as, for example, in a 2 liter flask with ground top to which a downwardly angled, air-cooled ground piece of large diameter was attached which was connected to a 2 liter receiver with ground top. There were obtained 820 grams of an ester which was only weakly yellowish colored and had the following characteristics:

|                                                      |                        |
|------------------------------------------------------|------------------------|
| Density at 20° C                                     | 0.905.                 |
| Refractive index, $n_D^{20}$                         | 1.4720.                |
| Molecular weight                                     | 432 (calculated: 432). |
| Pour point                                           | -28° C.                |
| Flash point                                          | 227° C.                |
| Viscosity at 50° C                                   | 2.17 Engler degrees.   |
| Viscosity index                                      | 140.                   |
| Color according to Ludwig-shafen iodine number scale | Below 4.               |
| Acid number                                          | 0.1.                   |
| Ester number                                         | 131 (calculated: 130). |
| Iodine number                                        | 57 (calculated: 59).   |
| Hydroxyl number                                      | 3.                     |
| Carbonyl number                                      | 0.                     |

To remove the low hydroxyl number still present, the ester described above, if desired, may be distilled once more as first runnings. This second distillation, however, is effected with the addition of 5-8 grams zinc oxide instead of magnesia. The purpose of adding magnesia in the first distillation is to combine the acid still present in the raw ester as, for example, p-toluene-sulfonic acid and small amounts of unesterified oleic acid. This results, however, in a slight ester cleavage which becomes evident in the ester distilled only once by the present hydroxyl number of 3. The addition of zinc oxide in the second distillation does not effect an additional ester cleavage but reduces the darkening of the color of the ester distillates. The change of the physical data of the ester by the removal of the hydroxyl number is only negligible.

#### Example 9

294 grams (1.75 mols) terpane methylol were esterified with 316 grams (1.93 mols) trichloroacetic acid with the addition of 2 grams p-toluene-sulfonic acid and 120 cc. benzene in the manner described in Example 8. After the termination of the water separation, the excess chloroacetic acid was removed from the esterification mixture by washing the same five times with water, and then the benzene added as the entraining agent for the water was driven off by distillation. The remaining raw ester was fractionated at about 5 mm. Hg. At 156°-158° C., an ester fraction was obtained which had the following characteristics:

|                              |                            |
|------------------------------|----------------------------|
| Density at 20° C             | 1.203.                     |
| Refractive index, $n_D^{20}$ | 1.4793.                    |
| Molecular weight             | 307 (calculated: 313.5).   |
| Chlorine content             | 33.5% (calculated: 34.1%). |
| Flash point                  | 160° C.                    |
| Pour point                   | -55° C.                    |
| Turbidity point              | -40° C.                    |
| Viscosity at 30° C           | 15.9 cst.                  |
| Viscosity at 80° C           | 3.59 cst.                  |
| Viscosity at 50° C           | 7.3 cst.                   |
| Viscosity index              | 135.                       |
| Color                        | Water-white.               |

#### Example 10

252 grams terpane methylol (1.5 mols) were esterified, in the manner described in the preceding example, with 151 grams pure lactic acid (1.68 mols) with the addition of 150 cc. benzene and 1.5 grams p-toluene-sulfonic acid. After the termination of the water separation, the excess lactic acid, similar to Example 9, was removed from the ester mixture by washing the same five times with water, and then the benzene was driven off. The remaining raw ester was fractionated at 10 mm. Hg. At a temperature between 160 and 173° C., a fractionated ester was obtained which had the following characteristics:

|                              |                        |
|------------------------------|------------------------|
| Density at 20° C             | 1.018.                 |
| Refractive index, $n_D^{20}$ | 1.4695.                |
| Molecular weight             | 238 (calculated: 240). |
| Flash point                  | 143° C.                |
| Pour point                   | -36° C.                |
| Turbidity point              | Not present.           |
| Viscosity at 30° C           | 37 cst.                |
| Viscosity at 50° C           | 13.4 cst.              |
| Viscosity at 80° C           | 4.65 cst.              |
| Viscosity index              | <-143.                 |
| Color                        | Water-white.           |
| Neutralization number        | 0.                     |
| Saponification number        | 229 (calculated: 233). |
| Hydroxyl number              | 229 (calculated: 233). |

We claim:

1. A low pour-point oil suitable as a low-temperature lubricating oil, comprising a monocarboxylic acid-monohydric alcohol ester having a terpane compound, obtained by the catalytic addition of carbon monoxide and hy-

drogen to the alkylene double bond of a terpene hydrocarbon containing an alkylene radical, as one of the monocarboxylic acid and monohydric alcohol components, and an aliphatic compound as the other component.

2. Process for the production of low pour-point oils, which comprises in combination the aldehydic catalytic addition of carbon monoxide and hydrogen to the aliphatic double bond of a terpene hydrocarbon containing an aliphatic radical with olefinic unsaturation to form the corresponding aliphatic aldehyde thereof, the treatment of said aldehyde with a member selected from the group consisting of oxygen and hydrogen to form the corresponding terpane carboxylic acid and terpane alcohol respectively, and the esterification of said terpane with an aliphatic compound, one of said terpane and aliphatic compound being a carboxylic acid and the other being an alcohol, and recovering an oil suitable as a low-temperature lubricating oil.

3. Process for the production of low pour-point oils, which comprises in combination the aldehydic catalytic addition of carbon monoxide and hydrogen to the alkylene double bond of a terpene hydrocarbon containing an alkylene radical to form the corresponding alkyl aldehyde thereof, the treatment of said aldehyde with a member selected from the group consisting of oxygen and hydrogen to form the corresponding terpane monocarboxylic acid and terpane monohydric alcohol respectively, and the esterification of said terpane with an aliphatic compound, one of said terpane and aliphatic compound being a monocarboxylic acid and the other being a monohydric alcohol, and recovering an oil suitable as a low-temperature lubricating oil.

4. A low pour-point oil suitable as a low-temperature lubricating oil, comprising a carboxylic acid-alcohol ester having a terpane compound, obtained by the catalytic addition of carbon monoxide and hydrogen to the aliphatic double bond of a terpene hydrocarbon containing an aliphatic radical with olefinic unsaturation, as one of the carboxylic acid and alcohol components, and an aliphatic compound as the other component.

5. Oil according to claim 4, in which said aliphatic compound contains from 2 to 20 carbon atoms.

6. Oil according to claim 5, in which said aliphatic compound is a branched chain monofunctional aliphatic compound containing more than 8 carbon atoms.

7. Oil according to claim 4, in which said ester is a terpane methylol-fatty acid ester.

8. Oil according to claim 4, in which said ester is a terpane carboxylic acid-aliphatic alcohol ester.

9. Process according to claim 2, in which said aliphatic compound contains from 2 to 20 carbon atoms.

10. Process according to claim 9, in which said aliphatic compound is a branched chain monofunctional aliphatic compound having a chain length of more than 8 carbon atoms.

11. Process according to claim 2, in which terpane methylol is esterified with a fatty acid.

12. Process according to claim 2, in which terpane carboxylic acid is esterified with an aliphatic alcohol.

13. Oil according to claim 5, in which said aliphatic compound contains from 4 to 18 carbon atoms.

14. Process according to claim 9, in which said aliphatic compound contains from 4 to 18 carbon atoms.

#### References Cited in the file of this patent

#### UNITED STATES PATENTS

|           |                |               |
|-----------|----------------|---------------|
| 900,316   | Shukoff        | Oct. 6, 1908  |
| 907,941   | Zietschel      | Dec. 29, 1908 |
| 969,420   | Sulzberger     | Sept. 6, 1910 |
| 2,501,199 | Wearn et al.   | Mar. 21, 1950 |
| 2,668,177 | Corbett et al. | Feb. 2, 1954  |
| 2,705,724 | Cottle et al.  | Apr. 5, 1955  |

#### OTHER REFERENCES

- Fieser et al.: *Organic Chemistry*, 1944, page 984.  
 Lo Cicero et al.: *J.A.C.S.*, vol. 74, No. 8, 1952, pp. 2094-2097.

Heilbron: *Dictionary of Organic Compounds*, 1953, page 826 (Norneole).